



US006363610B1

(12) **United States Patent**  
Narasimhan et al.

(10) **Patent No.:** US 6,363,610 B1  
(45) **Date of Patent:** Apr. 2, 2002

(54) **GAS TURBINE ROTOR BIMETALLIC RING SEAL AND METHOD THEREFOR**

(75) Inventors: **Dave Narasimhan**, Flemington; **Alexander S. Kozlov**, Wharton, both of NJ (US); **Steve H. Halfmann**, Chandler, AZ (US); **Mark C. Morris**; **Thomas E. Strangman**, both of Phoenix, AZ (US)

(73) Assignee: **Allied Signal, Inc.**, Morris Township, NJ (US)

(\*) Notice: Subject to any disclaimer, the term of this patent is extended or adjusted under 35 U.S.C. 154(b) by 0 days.

(21) Appl. No.: **09/422,587**

(22) Filed: **Oct. 21, 1999**

(51) Int. Cl.<sup>7</sup> ..... **B21D 53/84**

(52) U.S. Cl. ..... **29/888.3; 29/527.2**

(58) Field of Search ..... 29/888.3, 424, 29/527.2, 888.07, 888.074; 428/670, 936; 148/537; 277/654, 653, 650; 427/437, 405, 376.8, 376.6, 376.7

(56) **References Cited**

U.S. PATENT DOCUMENTS

3,635,586 A 1/1972 Kent et al.  
4,021,138 A 5/1977 Scalzo et al.  
4,432,555 A 2/1984 Langley

|             |         |                                      |
|-------------|---------|--------------------------------------|
| 4,477,087 A | 10/1984 | Sutter, Jr. et al.                   |
| 4,810,591 A | 3/1989  | Sakai                                |
| 4,916,022 A | *       | 4/1990 Solfest et al. .... 428/623   |
| 5,492,726 A | *       | 2/1996 Rose et al. .... 428/376.8    |
| 5,843,588 A | *       | 12/1998 Rose et al. .... 428/670     |
| 5,856,027 A | *       | 1/1999 Murphy .... 148/537           |
| 5,891,267 A | *       | 4/1999 Schaeffer et al. .... 148/537 |
| 5,942,337 A | *       | 8/1999 Rickerby et al. .... 428/670  |

FOREIGN PATENT DOCUMENTS

|    |        |         |
|----|--------|---------|
| JP | 80764  | 5/1984  |
| JP | 247386 | 10/1990 |

\* cited by examiner

Primary Examiner—I Cuda Rosenbaum

Assistant Examiner—T. Nguyen

(74) Attorney, Agent, or Firm—Robert Desmond, Esq.

(57) **ABSTRACT**

A method for making a bimetallic ring seal having a nickel core covered by a first layer of platinum having a inner dense portion and a second outer portion both of which plastically deform in the presence of a load. The method includes the step of applying a porous layer of platinum over the dense layer by electroless plating in a platinum bath comprising 0.8–1.2 gram/liter platinum as diammine dinitrite salt  $\text{Pt}(\text{NH}_3)_2(\text{NO}_2)_2$ , 50–100 milliliter/liter of 25% ammonium hydroxide  $\text{NH}_4\text{OH}$ ; and 0.3–1.5 gram/liter hydrazine hydrate  $\text{N}_2\text{H}_4\text{—H}_2\text{O}$ , at a temperature in the range of 75–90° C. and at a plating rate in the range of 0.5–3.0 micron/hour and then plastically deforming the ring seal under load.

11 Claims, 4 Drawing Sheets





FIG. 1 (PRIOR ART)



FIG. 2  
(PRIOR ART)



FIG. 3



FIG. 4



FIG. 5



FIG. 6

## GAS TURBINE ROTOR BIMETALLIC RING SEAL AND METHOD THEREFOR

### TECHNICAL FIELD

This invention relates to ring seals used in gas turbine engines and methods for making such ring seals. 5

### BACKGROUND OF THE INVENTION

A typical prior art ring seal used to seal between a seal plate and a turbine rotor in a gas turbine engine is shown in FIG. 1. Referring to this figure, a turbine rotor **10** consists of a wheel portion **12** which is coupled to other rotating components in the engine by curvic couplings **14**. In a manner familiar to those skilled in the art, at its radially outer periphery **16**, the rotor **10** has a plurality of circumferentially disposed fir-tree grooves. Each of these grooves receives a correspondingly shaped root of a blade **20**. The outer surface of the periphery **16** disposed between adjacent blades is referred to as a disk post **18**, which is shown in FIG. 2. A rotating seal plate **22** abuts the periphery **16** of the rotor **10**. Two conventional ring seals **24** are used to prevent leakage between the seal plate and the rotor. These seals are typically a simple split ring of nickel and are commonly used in gas turbine engines. 10 15 20

The blades **20** are usually mounted in the grooves at an angle that is offset from the axial axis of the engine. This angle is referred to as a broach angle. For highly loaded turbine rotors (i.e. those subject to high stresses due to high rotational speeds), the broach angle causes a net moment on the individual disk posts which may cause the posts to twist significantly. This twisting results in a sawtooth pattern between blades and disk posts as viewed from above and circumferentially around the rotor. For illustrative purposes, this sawtooth pattern is exaggerated in FIG. 2. The actual offset between the disk post and adjacent blades typically does not exceed 0.004 inches. Referring to this figure, because of the sawtooth pattern, triangular leakage areas **26** form between seal rings and the rotor periphery. Conventional nickel rings seals are not pliable enough to deform and fill these leakage areas resulting in a performance penalty to the engine. 25

Accordingly, there exists a need for a seal ring that is deformable so as to be able to fill these triangular leakage areas. 45

### SUMMARY OF THE INVENTION

An object of the present invention is to provide a deformable seal ring. 50

Another object of the present invention is to provide a method for making a deformable seal ring. 55

The present invention achieves this object by providing a ring seal having a nickel or cobalt core covered by a layer of a noble metal, preferably platinum. This layer further includes a dense inner layer and a porous outer layer both of which plastically deform in the presence of a load. 60

A method for making such a seal is also disclosed. The method starts with a nickel or cobalt wire ring and includes the following steps. 65

- coating said ring with a first layer of platinum to form a dense platinum layer;
- optionally heating said coated ring until said platinum and nickel diffuse together;
- applying a second layer of porous platinum over said first layer by electroless plating said coated ring in a plati-

num bath comprising 0.8–1.2 gram/liter platinum as diammine dinitrite salt  $\text{Pt}(\text{NH}_3)_2(\text{NO}_2)_2$ , 50–100 milliliter/liter of 25% ammonium hydroxide  $\text{NH}_4\text{OH}$ ; and 0.3–1.5 gram/liter hydrazine hydrate  $\text{N}_2\text{H}_4\text{H}_2\text{O}$ , at a temperature in the range of 75–90° C. and at a plating rate in the range of 0.5–3.0 micron/hour with the total thickness of the platinum layer being in the range of 0.002 to 0.006 inch. 70

heating said twice coated ring in an inert atmosphere until the included hydrogen in the porous platinum layer escapes creating a metallurgical bond between the core and the inner dense platinum layer and until the platinum is annealed, (i.e. softened); 75

cooling said twice coated ring and mounting said ring between said structures; and 80

plastically deforming the ring when placed under load in an engine or other application. 85

These and other objects, features and advantages of the present invention are specifically set forth in or will become apparent from the following detailed description of a preferred embodiment of the invention when read in conjunction with the accompanying drawings. 90

### BRIEF DESCRIPTION OF THE DRAWINGS

FIG. 1 is a cross-section of a turbine disk assembly that can employ a prior art ring seal or a ring seal contemplated by the present invention. 95

FIG. 2 is an illustration of a partial top view of the turbine disk assembly of FIG. 1 showing a prior art ring seal during engine operation. 100

FIG. 3 is a cross-section of the ring seal contemplated by the present invention before being mounted in an engine. 105

FIG. 4 is an illustration showing the ring seal of FIG. 3 after it is mounted in the turbine disc assembly of FIG. 1 and has plastically deformed during engine operation. 110

FIG. 5 is an illustration of a partial top view of the turbine disk assembly of FIG. 1 showing the ring seal contemplated by the present invention after it has plastically deformed during engine operation. 115

FIG. 6 is a flow chart illustrating a method for making the ring seal contemplated by the present invention. 120

### DESCRIPTION OF THE PREFERRED EMBODIMENT

FIG. 3 shows a ring seal **30** prior to being mounted in a turbine disc assembly. The seal **30** includes a nickel wire core **32** covered by a layer **34** of a noble metal with platinum being the preferred noble metal. The noble metal layer **34** includes a dense inner layer **36** and a porous outer layer **38**. In the preferred embodiment, the dense layer **36** is between 6–14 percent of the thickness of the layer **34** and more preferably 10 percent of this thickness. For highly loaded turbine rotors in the engine size class of 3,000 horsepower, a preferred nickel wire core **32** diameter is about 0.040 inches and a preferred platinum layer thickness **34** is about 0.003 inches. 125

Referring to FIG. 6, the ring seal **30** is fabricated as follows. First, a nickel wire is provided. Because nickel wire inherently is covered by an oxide layer, this layer is removed using mechanical cleaning methods familiar to those skilled in the art as well as an acid wash. (step **50**). Once cleaned, a thin layer of platinum, i.e. a few microns, is applied all around the outer surface of the nickel wire by conventional electroplating methods to form the dense layer **36**. (step **52**). Alternatively, the platinum can be applied by electroless

plating, sputtering, electron beam physical vapor deposition, or chemical vapor deposition. The coated wire is then placed in an oven and heated to 900–1000° C. for about 30 minutes. (step 54). This heating step is optional. During this heating step, the nickel diffuses into the platinum and the platinum diffuses into the nickel establishing a metallurgical bond. Next, additional porous platinum is added to the outer surface of the coated wire by electroless plating in a platinum bath. (step 56) with the total thickness of the platinum layer being in the range of 0.002 to 0.006 inch. In the preferred embodiment, the bath comprises 0.8–1.2 gram/liter platinum as diammine dinitrite salt  $\text{Pt}(\text{NH}_3)_2(\text{NO}_2)_2$ ; 50–100 milliliter/liter of 25% ammonium hydroxide  $\text{NH}_4\text{OH}$ ; and 0.3–1.5 gram/liter hydrazine hydrate  $\text{N}_2\text{H}_4\text{H}_2\text{O}$ . This step operates at a temperature in the range of 75–90° C. and at a plating rate of 0.5–3.0 micron/hour. More preferably, the bath comprises 1.0 gram/liter platinum as diammine dinitrite salt  $\text{Pt}(\text{NH}_3)_2(\text{NO}_2)_2$ ; 50 milliliter/liter of 25% ammonium hydroxide  $\text{NH}_4\text{OH}$ ; and 1.5 gram/liter hydrazine hydrate  $\text{N}_2\text{H}_4\text{H}_2\text{O}$ , with the temperature at 85° C. and a plating rate of 0.5 micron/hour at the beginning of the process and gradually increasing to 3.0 micron/hour as the surface area increases. After the electroless plating, the wire is heated in an inert atmosphere to between 900–1000° C. for about 30 minutes. (step 58). Due to the porous structure of the platinum layer, pathways are available for the included hydrogen to escape, (hydrogen outgassing), without forming disruptive hydrogen bubbles. Because bubbles do not form, the interface between the platinum and nickel is maintained without damaging the metallurgical bond.

After cooling to room temperature, (step 60), the ring seal 30 is ready for the final step of being mounted in the engine between the sealing plate and the turbine disc. (step 62). With additional reference to FIGS. 4 and 5, loads associated with high speed rotation of the seal plate force the wire seal 30 up between the disk periphery 16 and seal plate 22. Importantly, the seal 30 and in particular the porous platinum layer 34, plastically deform, (step 64), to permanently seal between the disc 10 and seal plate 22. As a result, the leakage triangles 26 that occurred with prior art ring seals are filled with plastic flow of the platinum layer 38 finally forming the ring seal 30 as contemplated by the present invention.

Though the invention has been described with respect to the preferred embodiment, it should be appreciated that this description of the invention should be considered exemplary and not as limiting the scope and spirit of the invention as set forth in the following claims.

What is claimed is:

1. A method for forming a ring seal for sealing between two structures comprising the steps of:
  - providing a ring made of a material selected from a group of nickel and cobalt;
  - coating said ring with a first layer of platinum to form a dense platinum layer;
  - applying a second layer of porous platinum having a thickness between about 0.002 inches to about 0.006 inches over said first layer by electroless plating;
  - heating said twice coated ring in an inert atmosphere until the included hydrogen escapes and a metallurgical bond forms between said core and said platinum;
  - cooling said twice coated ring and mounting said ring between said structures; and
  - plastically deforming the ring between said structures to form said ring seal.
2. The method of claim 1 further including between steps (b) and (c) the step of heating said coated ring in an inert atmosphere until said platinum and nickel diffuse together.

3. The method of claim 2 wherein said heating steps occur at a temperature in the range of 900–1000° C. for a period of about 30 minutes.

4. The method of claim 1 wherein in step (c) said coated ring is electroless plated in a platinum bath comprising 0.8–1.2 gram/liter platinum as diammine dinitrite salt  $\text{Pt}(\text{NH}_3)_2(\text{NO}_2)_2$ , 50–100 milliliter/liter of 25% ammonium hydroxide  $\text{NH}_4\text{OH}$ ; and 0.3–1.5 gram/liter hydrazine hydrate  $\text{N}_2\text{H}_4\text{H}_2\text{O}$ , at a temperature in the range of 75–90° C. and at a plating rate in the range of 0.5–3.0 micron/hour.

5. The method of claim 4 further including between steps (a) and (b) the step of cleaning said nickel wire.

6. The method of claim 4 further including in the electroless plating step, the step of varying the plating rate as the surface area increases.

7. A method for forming a ring seal for sealing between two structures comprising the steps of:

- providing a ring made from a material selected from a group consisting of cobalt and nickel;
- coating said ring with a first layer of platinum to form a dense platinum layer;
- applying a second layer of porous platinum having a thickness between about 0.002 inches to about 0.006 inches over said first layer by electroless plating said coated ring in a platinum bath comprising 1.0 gram/liter platinum as diammine dinitrite salt  $\text{Pt}(\text{NH}_3)_2(\text{NO}_2)_2$ , 50 milliliter/liter of 25% ammonium hydroxide  $\text{NH}_4\text{OH}$ , and 1.5 gram/liter hydrazine hydrate  $\text{N}_2\text{H}_4\text{H}_2\text{O}$ , with the temperature at 85° C. and a plating rate of 0.5 micron/hour at the beginning of the process and gradually increasing to 3.0 micron/hour as the surface area increases;
- heating said twice coated ring in an inert atmosphere until the included hydrogen escapes;
- cooling said twice coated ring and mounting said ring between said structures; and
- plastically deforming the ring between said structures to form said ring seal.

8. The method of claim 7 further including between steps (a) and (b) the step of cleaning said ring.

9. The method of claim 7 further comprising between steps (b) and (c) the step of heating said coated ring in an inert atmosphere until said platinum and nickel diffuse together.

10. The method of claim 9 wherein said heating steps occur at a temperature in the range of 900–1000° C. for a period of about 30 minutes.

11. A method for forming a ring seal for sealing between two structures comprising the steps of:

- providing a ring made from a material selected from a group consisting of cobalt and nickel;
- mechanically cleaning the ring such that the surface is substantially free from an oxide layer;
- coating said ring with a first layer of platinum to form a dense platinum layer;
- heating the coated ring in an inert atmosphere at temperature between about 900 to about 1000 degrees Celsius until the platinum and nickel diffuse together;
- applying a second layer of porous platinum having a thickness between about 0.002 inches to about 0.006 inches over said first layer by electroless plating said coated ring in a platinum bath comprising 1.0 gram/liter platinum as diammine dinitrite salt  $\text{Pt}(\text{NH}_3)_2(\text{NO}_2)_2$ , 50 milliliter/liter of 25% ammonium hydroxide  $\text{NH}_4\text{OH}$ , and 1.5 gram/liter hydrazine hydrate  $\text{N}_2\text{H}_4\text{H}_2\text{O}$ ,

H<sub>2</sub>O, with the temperature at 85° C. and a plating rate of 0.5 micron/hour at the beginning of the process and gradually increasing to 3.0 micron/hour as the surface area increases;

f) heating said twice coated ring in an inert atmosphere until the included hydrogen escapes;

- g) cooling said twice coated ring and mounting said ring between said structures; and
- h) plastically deforming the ring between said structures to form said ring seal.

\* \* \* \* \*